

## UNITED STATES PATENT OFFICE

2,298,918

## MODIFICATION OF FATTY OILS

László Auer, East Orange, N. J.

No Drawing. Application February 5, 1942,  
Serial No. 429,662

5 Claims. (Cl. 260—407)

## GENERAL FIELD OF INVENTION

This invention relates to the modification of organic isocolloids. More particularly, the invention is concerned with the bodying of fatty oils.

The subject matter claimed herein is divided from my copending application Serial No. 318,650 of which the present application is a continuation-in-part, and said subject matter is disclosed not only in said application 318,650 but also at least in part in certain other prior applications, especially Serial No. 359,425 (now Patent No. 2,213,944), and Serial No. 143,786 (now Patent 2,189,772).

Organic isocolloids are colloidal substances in which the dispersed phase and the dispersion medium are both of the same chemical composition, although present in a different physical state. In the bodying of fatty oils (which are organic isocolloids) the relation between the dispersed phase and the dispersion medium is altered, the dispersed phase being increased and the dispersion medium correspondingly decreased.

In accordance with various of my prior applications, including those mentioned above, various different methods are disclosed for modifying organic isocolloids, and especially for bodying fatty oils. In general, the modification is brought about by heating the isocolloid in the presence of a modifying agent.

In the prior applications, various different generic and sub-generic classes and specific modifying agents are disclosed; and, in addition, there are also disclosed variations in process. Different modifying agents or groups thereof, and also variations in process, effect different results, some being of importance for certain purposes and some for other purposes.

The present application is particularly concerned with the modification of fatty oils by means of polar compounds, i. e., modifying agents containing a positive charge in one part of the molecule and a negative charge in another part of the molecule, or capable of orienting their different radicals in opposite directions on an interface of liquid-gas, liquid-solid, or liquid-liquid. More specifically, the invention is concerned with that class of modifying agents which I have termed "2-radical" type, i. e., having within the

5 molecule an acidic inorganic residue and an organic residue. By an acidic inorganic residue I mean a residue capable of yielding an inorganic acid upon the addition of one or more hydrogen atoms or OH groups.

The subject matter claimed herein relates to the use of 2-radical type modifying agents in which the acidic inorganic residue is a nitrogenous residue and is capable of yielding an inorganic nitrogen-containing acid upon the addition of hydrogen or OH groups, for instance from a water molecule, this particular sub-group of agents having certain distinctive characteristics distinguishing it from other modifying agents in the general class, in which the inorganic radical does not contain nitrogen. The distinctive characteristics will be pointed out more fully hereinafter.

## THE STARTING MATERIAL

20 The fatty oils and similar materials with which the present application is especially concerned find one of their most important uses in the coating materials and plastics industries, especially the paint and varnish industry, where oils having good body and drying power are very important. The improved products produced in accordance with this invention also have many other uses.

25 A list of typical oils which may be advantageously modified by my invention is as follows:

|    |                       |               |
|----|-----------------------|---------------|
| 35 | Tung oil              | Rapeseed oil  |
|    | Castor oil            | Walnut oil    |
|    | Linseed oil           | Pine seed oil |
|    | Fish oil (train oils) | Corn oil      |
|    | Poppyseed oil         | Olive oil     |
|    | Sunflower oil         |               |

40 The ease of bodying or modification, under equal conditions, decreases in the order given. That is, the first mentioned oils are most extensively bodied or modified by my methods, while the oils at the end of the series are modified to a lesser body. However, it should be also mentioned that by the employment of suitable modifying agents in my methods, even the last mentioned oils (those at the end of this series) can be profoundly modified or bodied, as well as those oils appearing in the first of the series.

The foregoing listed, and other fatty oils may be classified as follows:

| Drying oils                                            | Semi-drying oils                                                                               |
|--------------------------------------------------------|------------------------------------------------------------------------------------------------|
| Tung oil<br>Oiticica oil<br>Linseed oil<br>Perilla oil | Sunflower oil<br>Poppyseed oil<br>Soya bean oil<br>Walnut oil<br>Rapeseed oil<br>Pine seed oil |
| Non-drying oils                                        | Special oils                                                                                   |
| Olive oil<br>Corn oil<br>Cottonseed oil<br>Coconut oil | Hydroxylated; castor oil, etc.<br>Fish oils (train oils)                                       |

The fish oils are mixtures of non-drying and drying triglycerides.

In accordance with the invention, the oils referred to may be treated per se, or they may be treated in mixtures containing more than one such oil, or containing other materials. For instance, synthetic resins containing natural resins or acids of fatty oils and of resins, may be modified in accordance with the invention.

In addition, separated fractions of fatty oils (for instance, the better drying fractions) may be used as starting materials, either alone or mixed with other oils.

The process of the present invention may, in fact, be used in connection with fatty oils themselves, fatty acids, esters of fatty acids, and various materials containing the same, and it is to be understood in connection with the appended claims that where reference is made to treating fatty oils, the language is not to be understood as limited to treatment of fatty oils per se, since essentially the same reaction takes place in the case of treatment of the fatty acids, esters thereof, etc.

#### THE MODIFYING AGENT

As hereinbefore mentioned, the present application is particularly concerned with the use of modifying agents having within the molecule an acidic inorganic nitrogenous residue, and an organic residue, the inorganic residue being capable, upon the addition of hydrogen or OH groups, of yielding an inorganic nitrogen-containing acid.

With reference to the yielding of a nitrogen-containing acid, it may be mentioned that although I believe that that reaction takes place during the treatment of the oil, in some cases the reaction may not occur to any considerable extent. Nevertheless, the treating agents herein contemplated are effective, so long as they have the capability of yielding the corresponding nitrogen-containing acid, upon the addition of hydrogen or OH groups to the inorganic residue.

In fuller explanation of the capability of yielding the nitrogen-containing acid, it is to be understood that the acid may be produced in different ways with different compounds. Thus, in some instances, the addition of OH groups is required, derived, for example, from  $H_2O$ . With some compounds the hydrogen or OH groups may be derived from other parts of the molecule of the treating agent itself (as by splitting off under application of heat), and with others one or the other, or both, of the hydrogen and oxygen may be derived from an external source, such as the treatment atmosphere or some materials present in the reaction. In any event, all of the materi-

als in question have in common the capability of yielding a nitrogen-containing acid.

Agents in this class are particularly effective for increasing the rate of bodying of oils, which may be due to the oxidizing nature of nitrogen compounds. One of the important uses for oils treated by these agents is employment thereof as bases for varnishes, especially water-resistant varnishes.

Still further, agents in the class here involved effect unusually extensive bodying of oils, in view of which the oil products are fast-drying. The products produced in accordance with the invention are, therefore, highly suitable for use in fast-drying water-resistant varnishes, for which there is a considerable field of utility.

Agents falling in the above group may be of a number of different types, the following being representative:

|    |                      |                       |
|----|----------------------|-----------------------|
| 20 | Nitrobenzene         | Dinitro-chlorobenzene |
|    | o-Nitrophenol        | Dinitroaniline        |
|    | p-Nitrophenol        | p-Nitro-acetanilide   |
|    | Dinitrobenzene       | 2:4-dinitrobenzene    |
|    | Nitro-chloro-benzene | Nitro-aminobenzene    |

25 Certain esters of inorganic acids have the important properties herein contemplated, for instance—

Nitrocresol carbonate

30 Again, some salts of organic bases function in accordance with the invention. For example—  
m-Nitroaniline hydrochloride

From the foregoing it will be seen that certain treating agents in the class herein claimed may be relatively complex compounds incorporating, in addition to the nitrogen-containing residue, other residues such, for instance, as a halogen-containing residue capable of yielding a halogen-containing acid upon addition of hydrogen, or a sulphur-containing residue capable of yielding a sulphur-containing acid upon addition of hydrogen or OH groups. In such cases, the treating agent partakes somewhat of the characteristics of the halogen or sulphur, as well as of the nitrogen-containing acid.

In this connection it is pointed out that in copending applications filed concurrently herewith (Serial Nos. 429,661 and 429,663), I have disclosed and claimed other 2-radical type treating agents having within the molecule a halogen-containing residue or a sulphur-containing residue. In certain instances, therefore, some of the treating agents herein referred to also belong to a group of agents claimed in a copending application, although in this event such a compound treating agent manifests not only the distinctive characteristic of the group claimed herein, but also the distinctive characteristic of the group claimed in said copending application.

#### TREATMENT CONDITIONS

In carrying out the process, the treating agent and the oil are first mixed together in any suitable way. Treating agents of different physical characteristics, such as consistency, naturally require different technique for mixing. These matters need not be considered in detail herein since they are fully disclosed in my copending application Serial No. 318,650.

The mixing may be effected in the cold, i. e., at room temperature; or may be effected at elevated temperatures, for instance at some temperature in the preferred range of reaction temperature.

While the quantity of treating agent may range

anywhere from a minor amount (for instance, a fractional percentage) up to about 30%, ordinarily the amount required is relatively small, not usually more than about 10%. In general, the degree of modification of the oil increases with increase in the amount of modifying agent used. The lower limit depends somewhat on the particular agent and also on the particular oil being treated, although at least some modification is observable from even minor fractional percentages, going down as low as .01%.

The treatment temperature may also be varied over a considerable range, depending upon the nature of the treating agent and of the oil, as well as on the character and extent of modification desired. In general, the temperature should be considerably above room temperature, but not above the boiling or decomposition point of the oil. A good working range is from about 100° to about 350° C., and preferably above about 200° C.

The time of treatment is also a variable, depending upon the treating agent, the starting material and the result desired. In general, increasing the time of treatment results in more extensive modification, and in most instances the treatment at reaction temperature should be continued for at least 30 minutes, and preferably for several hours.

The reaction may take place either in an open or in a closed vessel; and either at sub-atmospheric, at atmospheric, or at super-atmospheric pressure. Different results are secured under various of these conditions, as is brought out more fully in my copending application Serial No. 318,650.

With reference to the foregoing statement of treatment conditions, it is pointed out that these matters are discussed only briefly herein, since they are fully disclosed in my copending application Serial No. 318,650, to which reference may be had for further information. This is also true as to the supplemental matters discussed just below.

#### SUPPLEMENTAL TREATMENT CONDITIONS AND AGENTS

My processes may be practiced in the absence of any additional material, other than the polar compound. However, I have found it is advantageous in some cases to incorporate the polar compound in the presence of additional materials which facilitate its incorporation and the modification of the organic isocolloid. For instance, the polar compound may be incorporated in the presence of various organic bodies such as the purely organic additions mentioned post or organic solvents. Again metal soaps may also be added; for instance siccatives (driers) such as the resinites and linoleates of metal compounds and metal oxides, commonly used in the varnish industry, as is mentioned in Serial No. 143,786. Further, sulphur or sulphur compounds, such as sulphur chloride, etc., may also be used in these processes and added in addition to the polar compound during the reaction or as an after treatment. The sulphur or sulphur compounds effect further modification and produce sulphurized products. The temperature usually employed for modification (above 200° C.) being substantially above normal vulcanization temperatures, the effect of the sulphur treatment at modifying temperatures is quite different from vulcanization.

However, I may also effect vulcanization of my modified products in an after treatment, so as to

product solid, coherent and elastic products, similar in some characteristics to ordinary rubber. Sulphur may be used for this purpose and may be added as such, or in the form of a sulphur compound, such as sulphur chloride, etc. The action of the sulphur is analogous to that which takes place in the vulcanization of rubber. Thus, accelerators or activators (zinc oxide, etc.) or both, such as usually employed in the vulcanization of rubber, may be used in my processes to accelerate vulcanization when sulphur, etc. is added. The added sulphur vulcanizes or sulphurizes my modified products further changing their properties.

When making solid vulcanized rubber-like products, I employ temperatures between 120° and 180° C. for vulcanization, and from 5 to 50 parts of sulphur to 100 parts of the isocolloid under treatment. This vulcanization should be effected after modification, and accelerators and antioxidants may be added to the mix in known manner. I may produce liquid vulcanized products as well as rubber-like solids, by regulating the amount of sulphur and the time and temperature of heating. The liquid products are useful as varnish or paint bases.

Two step methods for making vulcanized, modified, heat-bodied fatty oil products are described and claimed in my application Serial No. 236,800 (Patent 2,234,545). As there stated, many of those products are useful as "rubber substitutes." Others are useful for other purposes, for instance, in the manufacture of varnishes, lacquers and other liquid coating compositions, as well as in plastic compositions.

As noted above, the processes may be carried out in various ways, for instance, either in open or closed vessels as desired. In the latter case, the air can be entirely or partially displaced by another gas, such as hydrogen, CO<sub>2</sub>, SO<sub>2</sub>, H<sub>2</sub>S, nitrogen, etc., which influence the results obtained, these gases being used in supplement to the primary modifying agent employed. Again, in both cases such gases may be passed through the material being treated. That is, the modification can be carried out during the passage of a gas. The gas pressure can be that of atmospheric. In many cases, however, a vacuum may be used with advantage. Again, even a higher pressure, of several atmospheres is to be recommended in certain cases, it being sometimes advantageous.

That is, I have further found that the results of the process vary with the nature of the gas present and also with the physical condition (pressure) of this gas. Thus I have found that a certain given starting material which is initially liquid will become slightly viscous only as a result of the modifying treatment, if the latter is effected under atmospheric pressure (open vessel) but more viscous if the gas is rarefied by the employment of a partial vacuum. In other cases the converse applies. When plus pressure was used the results differ again. Air gives a different result from another gas or mixtures of gases such as mentioned ante. The modifying treatment may be carried out either in the total or partial absence of air, by replacing the same with another gas, such as those shown ante.

A pressure treatment followed by a vacuum treatment may be used, and I have found it to be advantageous to use alternately, atmospheric or plus pressure and vacuum treatment. Such alternate treatment increases the uniformity of the distribution of the polar compound in the

organic isocolloid. In my processes, the gas may be blown or passed through the liquid mass or simply passed over the surface of the same during the heating. It is advisable in some cases, both when open or closed vessels are employed to have a constant passage of the gas, such as those given ante, during the treatment with polar compound.

It may be stated with reference to the action of gases, that generally speaking rarefaction of the gases present, by reduction of pressure in the vessel in which the treatment is given, tends to intensify the action of the gases in my processes.

If desired, the polar compound may be produced in situ, that is, within the organic isocolloid under treatment, by interaction within the organic isocolloid, of substances capable of reacting under the conditions of the process to reduce the polar compound. The same applies to the gas in the presence of which the organic isocolloid is to be treated and a substance or substances may be added which evolve the desired gas during the processing. It has been found in certain cases that polar compounds and gases which are produced in situ, being in the nascent state, are somewhat more active than those added in the pre-formed state.

Likewise, the organic isocolloid itself may be formed in situ during the treatment. That is, if it is desired to modify an organic isocolloid which is not a naturally occurring material and which has to be produced before it can be treated, the production of such artificial or manufactured organic isocolloid may be advantageously combined with the treatment with the polar compound. For instance, in making modified heat-bodied fatty oils, the oil may be both heat-bodied and modified in a single step by heat-bodying the fatty oil in the presence of the electrolyte or polar compound. To do this several hours heating at polymerization temperatures is required. Many of my polar compounds are advantageous for this purpose as they accelerate the heat-bodying and polymerization of fatty oils.

In addition to the action of polar compounds and the cooperating action of gases in effecting the colloidal transformations characteristic of my invention, an additional modification of the ultimate physical properties of the treated products can be effected by the addition to the material under treatment, of purely (i. e. metal-free) organic bodies, such as phenols, naphthols, naphthalene, chloroform, acetone, alcohols and their homologues and derivatives. These additions are supplemental to the use of polar compounds. Some of them are solvents and assist in dispersing the polar compound in the organic isocolloid. The use of solvents for this purpose is also shown in my Serial No. 273,159 (Patent 1,985,230) and other prior applications.

I have also found that in my processes the colloidal transformations may be promoted by the use of rays of oscillating energy, such as ultra-violet rays, infra-red rays, X-rays, etc. That is, it is advantageous to irradiate the oil or other organic isocolloid, before or during the treatment with the polar compound. Sometimes a subsequent treatment with these rays is also helpful. Further, these rays influence and intensify the action of the gases in my processes.

#### EXAMPLES

##### Example 1

300 parts of linseed oil are heated with 15 parts

of p-nitroacetanilide in a vacuum to 280-310° C. for 5 hours. The modified oil product so obtained is a soft solid, moderately dark in color. It can be advantageously used in preparing varnishes and like coating compositions.

#### Example 2

##### COMPARATIVE TESTS

Whereas profound changes in physical properties of fatty oils usually require modifying agents in quantities of 1% or more, gradual changes of properties, such as bodying velocity, may be brought about with smaller proportions of modifying agent. Several comparative tests were carried out, using .5% of modifying agent. In each instance the oil treated was alkali refined linseed oil.

In each test a batch of 300 grams of oil in a 1 liter aluminum beaker was heated at atmospheric pressure (the beaker being open) to 295° to 305° C. and kept at that temperature for 5 hours. Two modifying agents were tried in this way and a blank control experiment was also carried out, following the same heating procedure, in order to secure a comparison between the linseed oil, heat bodied with and without modifying agent. Color and viscosity of the oils were as follows:

| Reagent                     | Color of oil | Viscosity of oil |
|-----------------------------|--------------|------------------|
| Blank                       |              |                  |
| Alpha-nitroso-beta-naphthol | 7            | X                |
| Nitroanthraquinone          | 16<br>12+    | Z-2<br>Z-6       |

Readings of both color and viscosity are on the Gardner scale.

Each of the above oils was further used in preparing a varnish, as follows:

40 2 parts of oil product and 1 part of ester gum were heated to 300° C. and kept at that temperature for 1 hour. The mixture was cooled to 200° C. and thinned with 3 parts of mineral spirits to 50% solids. Naphthenate driers were added in the proportion of .03% cobalt metal, .02% manganese metal and .3% lead metal, based on the quantity of oils used.

45 The color and viscosity of the varnish in each case was as follows:

| Reagent                     | Color of varnish | Viscosity of varnish |
|-----------------------------|------------------|----------------------|
| Blank                       |                  |                      |
| Alpha-nitroso-beta-naphthol | 11               | A                    |
| Nitroanthraquinone          | 14<br>18+        | A<br>A               |

50 The foregoing varnishes were stored for 2 days and then panels of steel were coated with a coating knife yielding heavy films of .003" thickness.

Various characteristics of the varnishes were tested, with the following results:

| Reagent                     | Initial drying | Over-night tack-freeness | Cold water resis. | Boiling resis. | Alkali resis. (3% alk.) |
|-----------------------------|----------------|--------------------------|-------------------|----------------|-------------------------|
| Blank                       | F              | VG                       | F                 | B              | F                       |
| Alpha-nitroso-beta-naphthol | VG             | VG                       | VG                | F              | G                       |
| Nitroanthraquinone          | G              | VG                       | VG                | VG             | VG                      |

VG = very good.

G = good.

F = fair.

B = bad.

The "initial drying" indicates an observation made after the first 5 hours of drying. "Overnight tackfreeness," of course, indicates the condition after overnight drying. Before subjecting the panels to the cold water, boiling water and alkali resistance tests they were left to through-dry for 48 hours. All of the immersion tests were made in a manner leaving one-half of the panels exposed, for comparative purposes.

The cold water test was made by immersing the panels for 24 hours in cold water and observing the appearance of the film.

The boiling water test was made by immersing the panels in boiling water for 15 minutes, and comparing the results. In this case the degree of milkiness and softness of the films was observed as well as the speed with which the milky films returned to their original appearance upon air drying.

The alkali resistance test was made by immersing the panels in a 3% sodium hydroxide solution and noting the time when the alkali completely attacked and dissolved the films.

#### Examples 3-7

In another series of comparative experiments, certain uniform treatment conditions were adopted, as follows:

In each case the oil employed was linseed oil and 5% of the treating agent was used.

In each case the heating time was in the neighborhood of 5 hours. In conducting these experiments the appropriate reaction temperature was 300° C., although there were minor differences between various of the experiments. The treatment temperature was between about 290° to 310° C.

A control experiment was also conducted under the same heating conditions, but without treating agent, so as to secure comparative results.

The experiments in this group may be divided into pairs, the two experiments of each pair employing the same treating agent. The difference between the treatment of the two members of each pair was as follows:

1. Heating a 300 gram charge in a 1 liter distilling flask under vacuum—identified herebelow by the letter (a) following the example number.

2. Heating a 150 or 300 gram charge in a 500 cc. open enameled beaker—identified herebelow by the letter (b) following the example number.

#### Example 3(a)

##### *o-Nitrophenol*

The reagent dissolved at about 81° C. During rise in temperature some bumping and slight volatilization took place. At treatment temperature the mixture boiled steadily, and after about 2 hours began to thicken, reaching an almost solid condition. Additional heating caused some thinning. The product was a black sticky mass, which was somewhat plastic.

#### Example 3(b)

##### *o-Nitrophenol*

Some boiling occurred during rise in temperature and the mixture then subsided. In addition a small amount of reagent sublimed at about 240° C. Boiling took place throughout most of the time on temperature.

The product was a highly viscous sticky liquid, dark brown in color, with a green appearance in reflected light.

#### Example 4(a)

##### *Dinitroaniline*

On initial rise in temperature the mixture frothed slightly but then subsided, and at about 240° C. gas was evolved and some distillation took place. Distillation ended shortly after reaching treatment temperature and the mixture began to thicken in about 3½ hours, at which time some explosions occurred within the mixture. Toward the end of the treatment time the mixture again commenced to thin so that the product was poured out after about 4 hours and 20 minutes.

The product was a semi-solid dark brown elastic mass.

The distillate settled in two layers, the bottom layer being clear and the top layer a red oil.

#### Example 4(b)

##### *Dinitroaniline*

During rise in temperature yellow fumes were evolved and a sample spotted showed the mixture to be a thick dark brown oil. Treatment temperature was reached in about 1 hour, at which time the fumes had subsided. After about 2 and ½ hours on temperature the mixture had jelled. Continued heating showed no signs of thinning and the mixture was then poured out, an explosion occurring when pouring the last portions.

The product was a black rubbery jelly.

#### Example 5(a)

##### *p-Nitrophenol*

The mixture very promptly frothed, but after reaching about 180° to 190° C. the frothing subsided and a very vigorous reaction took place, lasting some two or three minutes. The mixture commenced to boil steadily at about 293° C. and this was continued for 2½ hours. Continued heating caused distillation.

The product was a semi-solid dark brown elastic mass.

The distillate subsided and formed two layers, the bottom layer being about 1 cc. of a faint yellow liquid and the top layer about 20 cc. of dark red oil.

#### Example 5(b)

##### *p-Nitrophenol*

On initial heating frothing occurred but this promptly subsided and at about 296° C. yellow fumes were evolved. The product was a very thick sticky dark brown oil with a dull green fluorescence.

#### Example 6(a)

##### *p-Nitro acetanilide*

Bad frothing occurred during initial rise in temperature and distillation of reagent also set in. The temperature was kept below about 200° C. for 1½ hours to prevent loss of reagent. Gentle boiling occurred on temperature.

The product was a black sticky semi-solid mass.

#### Example 6(b)

##### *p-Nitro acetanilide*

Slight frothing occurred on initial heating, but this rapidly subsided. The mixture darkened and thickened while on temperature.

The product was brown in color and of the consistency of treacle.

## Example 7(a)

*p*-Nitro chlorobenzene

Boiling set in at about 250° C. and some bumping followed shortly. However, on temperature 5 the mixture soon subsided.

The product was a fairly viscous oil of dark brown color.

## Example 7(b)

*p*-Nitro chlorobenzene

The reagent dissolved rapidly on warming the oil and the oil gradually darkened as it approached the reaction temperature.

The product was a brown fluorescent oil—15 somewhat thinner than the product of Example 7(a).

The data relating to Experiments 3 to 7 inclusive is given herebelow in tabular form for purposes of ready comparison. The table also 20 indicates characteristics of the blank control experiment.

| Example                      | Viscosity             | Color                   | Reagent solubility                   |
|------------------------------|-----------------------|-------------------------|--------------------------------------|
| 3(a)—V                       |                       |                         |                                      |
| <i>p</i> -Nitroacetanilide   | Medium soft (solid)   | Fairly dark             |                                      |
| 3(b)—B                       |                       |                         |                                      |
| <i>p</i> -Nitroacetanilide   | Med. viscous (liquid) | Light (medium)          |                                      |
| 4(a)—V                       |                       |                         |                                      |
| <i>o</i> -Nitrophenol        | Soft solid            | Fairly dark             | Dissolves in 5 min. at 80° C.        |
| 4(b)—B                       |                       |                         |                                      |
| <i>o</i> -Nitrophenol        | do                    | do                      | Dissolves in 5-10 min. below 100° C. |
| 5(a)—V                       |                       |                         |                                      |
| Dinitraniline                | do                    | do                      |                                      |
| 5(b)—B                       |                       |                         |                                      |
| Dinitraniline                | do                    | do                      |                                      |
| 6(a)—V                       |                       |                         | Part undissolved.                    |
| <i>p</i> -Nitrophenol        | Thick viscous (fluid) |                         |                                      |
| 6(b)—B                       |                       |                         | Do.                                  |
| <i>p</i> -Nitrophenol        | Soft solid            | Fairly dark             |                                      |
| 7(a)—V                       |                       |                         |                                      |
| <i>p</i> -Nitrochlorobenzene | Med. viscous (liquid) | Medium (greenish-brown) | Dissolves.                           |
| 7(b)—B                       |                       |                         |                                      |
| <i>p</i> -Nitrochlorobenzene | do                    | Light (med. greenish)   | Do.                                  |
| Blank                        | Thin viscous (liquid) | Light                   |                                      |

## Code explanation:

V = vacuum experiment.

B = open beaker experiment.

Viscosity = range from heavy to light.

Color = range from dark to light.

Varnishes were made up employing the products of Experiments 3 to 7, the varnishes being without driers. The relative drying order of the varnishes is indicated in the following list:

| Example No. | Drying order of varnish (no driers) |
|-------------|-------------------------------------|
| 3 (a)       | 3                                   |
| 3 (b)       | 9                                   |
| 4 (a)       | 1                                   |
| 4 (b)       | 2                                   |
| 5 (a)       | 11 70                               |
| 5 (b)       | 5                                   |
| 6 (a)       | 4                                   |
| 6 (b)       | 6                                   |
| 7 (a)       | 10                                  |
| 7 (b)       | 8                                   |
| Blank       | 7                                   |

The best drying was the varnish made with the product of Example 4(a), the others following in sequence as indicated.

I claim:

1. In the modification of fatty oils to improve their drying properties, the process which comprises mixing the oil with a minor amount and not more than 10% of a polar compound having within the molecule an organic residue, and an 10 acidic inorganic nitrogenous residue capable of yielding a nitrogen-containing acid, and heating the mixture to a reaction temperature between about 200° and 350° C. for at least thirty minutes.

2. In the modification of fatty oils to improve their drying properties, the process which comprises mixing the oil with a minor amount and not more than 10% of an organic nitro- compound, and heating the mixture to a reaction temperature between about 200° and 350° C. for at least thirty minutes.

3. A process in accordance with claim 2 in

which said nitro- compound is a benzol derivative.

4. A process in accordance with claim 2 in which the nitro- compound is a naphthalene derivative.

5. A process in accordance with claim 2 in which the fatty oil is linseed oil.

LÁSZLÓ AUER.